

## UNITED STATES PATENT OFFICE

2,429,198

## CUTTING OIL COMPOSITION

Louis H. Sudholz and Cecil D. Flemming, New York, N. Y., assignors to Socony-Vacuum Oil Company, Incorporated, a corporation of New York

No Drawing. Application June 8, 1944,  
Serial No. 539,390

3 Claims. (Cl. 252—48.6)

1

This invention relates to an improved cutting oil composition containing sulfurized taloil and free from deposition of sludge.

U. S. Patent 2,198,562, "Method of making sulfurized cutting oils," to Arthur Pollak and Randall Hastings, assignors to West Virginia Pulp & Paper Company, discloses that the use of sulfurized taloil, cut back with other oils such as mineral oils, presents some difficulty in that "ordinarily the sulfurized oil deposits a sludge upon standing which detracts from the usefulness of the oil for cutting purposes." A method is given wherein the resultant sludge deposition is kept at a minimum. This method consists in using a refined taloil and sulfurizing it at controlled conditions of time and temperature, namely from 2 to 4 hours, within a temperature range of 300° F.—400° F. However a certain amount of sludge still separates from mineral oil blends, both paraffinic and asphaltic, upon standing, as admitted in the patent specification. This deposit being quite gummy and sticky adheres to the metal surfaces of the lathe, tools and pump parts, thus preventing their normal operation.

The above drawbacks have been confirmed in experiments. When a blend of 6% of sulfurized refined taloil (Indusoil) and 94% of pale paraffin oil was installed in a test lathe for purposes of evaluation of the sulfurized base, after standing in the machine tool over the week end, the coolant pump was so badly gummed up that it was necessary to disassemble it for cleaning. The ways of the lathe were coated with a sticky film which prevented the passage of the carriage. A similar blend, installed in pipe threading machine for

5 evaluation in the threading of a 2 inch seamless steel tubing showed that a large amount of sludge separated out overnight, the sticky mass adhering to the machine tool parts and being difficult to remove.

The sulfurized taloil used in the above experiments was made from refined taloil and in accordance with the teachings of the Pollak-Hastings patent.

- 10 This invention is based upon the discovery that the addition of aromatic solvents to cutting oils containing sulfurized taloil prevents separation of sludge, and in extreme cases of slight separation, the sludge is of such a nature that it does not adhere to the metal surfaces. The aromatic solvents used in the experimental work were 15 those derived from high temperature catalytic conversion of petroleum oils, specifically those derived from recycle stocks from catalytic cracking. Characteristics of solvents used are given 20 below.

|                                | Medium<br>Aromatic<br>Solvent | Heavy<br>Aromatic<br>Solvent |
|--------------------------------|-------------------------------|------------------------------|
| 25 Grav. ° API                 | 12                            | 3                            |
| Spec. Grav. @ 60°/60°          | .985                          | 1.05                         |
| Flash Pt. COC, ° F.            | 265                           | 335                          |
| Aniline Pt., ° F.              | —20                           | —25                          |
| 30 Approx. Boiling Range, ° F. | 500-600                       | 600-700                      |

35 Experimental data are tabulated below. In all blends listed, the sulfurized taloil was made by sulfurizing "Indusoil" (refined taloil) to a 15% sulfur content at a temperature of about 350° F.

Table I

| Blend                            | Stability of Blend              |                                                                                            |
|----------------------------------|---------------------------------|--------------------------------------------------------------------------------------------|
|                                  | After Standing 1 week           | After Standing 5 weeks                                                                     |
| 3% Sulfurized Tallow             | Cloudy, appreciable separation  | Almost all of sulf. taloil separated out (adhesive deposit).                               |
| 97% 100% paraffin oil            | do                              | Clear, large amount of separated material (adhesive material).                             |
| 6% Sulfurized Tallow             | do                              | Large amount of separated material (adhesive material).                                    |
| 94% 100% paraffin oil            | do                              | Appreciable separation.                                                                    |
| 9% Sulfurized Tallow             | do                              | Slight separation (deposit not adhesive).                                                  |
| 91% 100% paraffin oil            | do                              | Clear, trace of separation (material which separated out not adhesive. Readily dispersed). |
| 3% Sulfurized Tallow             | Cloudy, slight separation       | Clear, trace of separation (material which separated out not adhesive. Readily dispersed). |
| 5% Med. Aro. Solvent             | do                              | Clear, trace of separation (material which separated out not adhesive. Readily dispersed). |
| 92% 100% paraffin oil            | do                              | Cloudy, considerable separation.                                                           |
| 3% Sulfurized Tallow             | Cloudy, slight separation       | Slight separation, Sticky deposit.                                                         |
| 10% Med. Aro. Solvent            | Cloudy, slight separation       | Trace of separation—material separated out not adhesive, readily dispersed.                |
| 87% 100% paraffin oil            | do                              |                                                                                            |
| 3% Sulfurized Tallow             | Clear, trace of separation      |                                                                                            |
| 15% Med. Aro. Solvent            | do                              |                                                                                            |
| 82% 100% paraffin oil            | do                              |                                                                                            |
| 6% Sulfurized Tallow             | do                              |                                                                                            |
| 15% Med. Aro. Solvent            | do                              |                                                                                            |
| 79% 100% paraffin oil            | do                              |                                                                                            |
| 6% Sulfurized Tallow             | Cloudy, much separation         |                                                                                            |
| 94% 100% paraffin oil            | do                              |                                                                                            |
| 3% Sulfurized Tallow             | Cloudy, considerable separation |                                                                                            |
| 97% 100% Coastal (Asphaltic) Oil | Cloudy, considerable separation |                                                                                            |
| 6% Sulfurized Tallow             | Slight separation               |                                                                                            |
| 94% 100% Coastal (Asphaltic) Oil | do                              |                                                                                            |
| 6% Sulfurized Tallow             | do                              |                                                                                            |
| 15% Med. Aro. Solvent            | do                              |                                                                                            |
| 79% 100% Coastal Oil             | do                              |                                                                                            |

It will be seen from the above data that the incorporation of 10% or more of the aromatic solvent produced cutting oils satisfactory from the standpoint of stability and freedom of sludge deposition, whereas blends of sulfurized taloil with either paraffinic or asphaltic oils invariably failed in that respect. Even in cases when some separation was observed with smaller additions of the aromatic solvent, the sludge was not adhesive to metal and was readily dispersed by slight movement of the oil. It is believed that this constitutes an improvement which makes the sulfurized taloil blends suitable for operation in cutting machines.

Supplementary experimental work was conducted to check the performance of the improved taloil cutting oils containing the aromatic solvents in actual service. The following cutting oil was prepared.

|                                        | Percent |
|----------------------------------------|---------|
| Sulfurized refined taloil (15% sulfur) | 6       |
| Hy. Aro. solvent                       | 15      |
| 100% paraffin oil                      | 79      |

The above product was evaluated in the threading of 2 inch seamless steel tubing and left in the machine over night. No sticky resinous deposit was observed on parts of the machine tool or on the work. The oil was drained from the machine into an iron pail and allowed to stand for several days. No instability of the oil was indicated.

The metal cutting efficiency of the above blend was compared with that of a conventional sulfurized fat base cutting oil. The latter contained the same percent of sulfur, in the base and in the finished cutting oil. The threading efficiency of the two products under comparison, as expressed in kilowatts or specific power consumption was the same. This indicates that the performance of the stabilized sulfurized taloil blend compared favorably with blends of conventional sulfurized fat bases.

The aromatic oils used for this stabilization are in general derived from the high boiling portions of a material which has been subjected to severe cracking and find no counterpart in uncracked oils of similar boiling point. The nature of the oils to be used may be noted from the following table of properties defining oils useful for the purpose.

Table II

|                                       |             |
|---------------------------------------|-------------|
| Sp. gravity @ 60/60° F.               | .90-1.06    |
| Flash (C. O. C.) °F.                  | 250 minimum |
| Viscosity Saybolt Universal @ 100° F. | 30-200 sec. |
| Aniline point, °F.                    | +40 max.    |
| Refractive index @ 20° C.             | 1.50 min.   |
| Initial boiling point, °F.            | 450 min.    |

Most striking of these properties is the combination of viscosity and gravity, wherein the

combination of low viscosities, (30-200° S. U. V. @ 100° F.), with high gravities (.97-1.06), (as heavy as water, practically), indicates an oil of a nature quite different from those found in ordinary lubricants, either distillate or residual.

These oils should be incorporated into the final composition to the extent of from 5% to 30% of the final composition, the preferable range being from 10% to 20%, and the apparent optimum being about 15%.

We claim:

1. A sulfurized taloil cutting oil composition stable against the formation of sludge comprising a mineral oil lubricating fraction, a sulfurized taloil, and from about 5% to about 30% of a hydrocarbon oil having an aniline point of +40° F. or lower, a specific gravity of from 0.9 to 1.06, a flash point of 250° F. minimum, an initial boiling point of not less than 450° F., and a viscosity of not over about 200 seconds Saybolt Universal at 100° F.

2. A sulfurized taloil cutting oil composition stable against the formation of sludge comprising a mineral oil lubricating fraction, a sulfurized taloil, and from about 10% to about 20% of a hydrocarbon oil having an aniline point of +40° F. or lower, a specific gravity of from 0.9 to 1.06, a flash point of 250° F. minimum, an initial boiling point of not less than 450° F., and a viscosity of not over about 200 seconds Saybolt Universal at 100° F.

3. A sulfurized taloil cutting oil composition stable against the formation of sludge comprising a mineral oil lubricating fraction, a sulfurized taloil and about 15% of a hydrocarbon oil having an aniline point of +40° F. or lower, a specific gravity of from 0.9 to 1.06, a flash point of 250° F. minimum, an initial boiling point of not less than 450° F., and a viscosity of not over about 200 seconds Saybolt Universal at 100° F.

LOUIS H. SUDHOLZ.  
CECIL D. FLEMMING.

#### REFERENCES CITED

The following references are of record in the file of this patent:

#### UNITED STATES PATENTS

| Number       | Name             | Date          |
|--------------|------------------|---------------|
| 50 2,031,986 | Stratford        | Feb. 25, 1936 |
| 2,128,109    | Wiezevich        | Aug. 23, 1938 |
| 2,198,562    | Pollak           | Apr. 23, 1940 |
| 2,202,501    | Magill           | May 28, 1940  |
| 2,281,894    | von Fuchs et al. | May 5, 1942   |
| 2,363,880    | Lieber           | Nov. 28, 1944 |

#### OTHER REFERENCES

American Mineral Spirits Co. publication (U. S. Patent Office Library), Jan. 9, 1943.